

# UNITED STATES PATENT OFFICE.

ROBERT NASSE, OF ST. PAUL, MINNESOTA, ASSIGNOR OF ONE-HALF TO AUGUST PROHOF SKY, OF ST. PAUL, MINNESOTA.

## PROCESS IN TANNING FUR SKINS.

1,210,968.

Specification of Letters Patent. Patented Jan. 2, 1917.

No Drawing.

Application filed January 3, 1916. Serial No. 69,776.

To all whom it may concern:

Be it known that I, ROBERT NASSE, a citizen of the United States, residing at St. Paul, in the county of Ramsey and State of Minnesota, have invented a new and useful Improvement for a New Process in Tanning Fur Skins, of which the following is a specification.

This invention relates to the process of 10 tanning fur skins, by means of a tanning solution composed of aluminum potassium sulfate, sodium chlorid, sodium borate, and water, and a solution composed of wheat flour, brewers' yeast, alcohol, and water, and has for its object to make the process more 15 expeditious and give a skin which is softer and more full of life when tanned.

Heretofore in tanning fur skins with a 20 solution of aluminum potassium sulfate, sodium chlorid, etc., the skin needed considerable working with oil and other fat elixers to soften them after the tanning process, and even then, they would not always be soft and pliable. With the old process of 25 tanning, the skins seemed to deteriorate rapidly after being tanned, while with my process, the skins remain the same and seem to retain the life and softness.

In my process of tanning I use a solution 30 made up of ingredients in the proportions approximately as follows: aluminum potassium sulfate 100 pounds, sodium chlorid 80 pounds, sodium borate 3 pounds and 25 gallons of water. I then make up a second solution of ingredients and proportions approximately as follows: wheat flour 100 pounds, brewers' yeast 1 pound, alcohol one pint and adding water to make 28 gallons. The solution of wheat flour, yeast, alcohol and water 35 is left to ferment about two days before using.

For convenience I term the first solution of aluminum potassium sulfate, sodium chlorid and water, the mineral tanning solution, and the second solution composed of 45 wheat flour, yeast, alcohol and water the organic solution.

In the process of tanning, I take about 8 gallons of the mineral tanning solution and 50 add sufficient water to make a ten per cent. solution, to which I add 4 gallons of the organic solution and about 10 pounds of bran, then applying this solution on the flesh side of the skins and place them flesh

to flesh to remain in this way for 12 hours 55 which is sufficient time to tan the skins. In the process of tanning the fermented solution, which is mixed with the tanning solution, takes away some of the coriin, thus leaving the fiber looser and allowing more 60 perfect action of the tanning liquor. It being an undoubted fact that the bacteria in the fermented solution feed upon the hide substance.

By my improved process, the skins are 65 very much finer in quality and the length of time for finishing the same is materially reduced, such as in the saving of working the skins to soften them after they have been 70 tanned.

If it is desired to have a thin leather on the skins, I treat the same with a solution of mild white soap and water which is boiled together and left to stand for some time before using. This soap solution is applied 75 warm with any good fur oil and the skins placed flesh to flesh after this solution has been applied and left for several hours.

Having described my invention, what I 80 claim is:

1. The process of tanning fur skins consisting in treating the skins with a solution of aluminum potassium sulfate, sodium chlorid, sodium borate and water, mixed with a solution of wheat flour, brewers' 85 yeast, alcohol and water, in about the proportions specified.

2. The process of tanning fur skins consisting in treating the skins with a solution of aluminum potassium sulfate, sodium 90 chlorid, sodium borate and water, mixed with a fermented organic solution of the ingredients named in about the proportions specified.

3. The process of tanning fur skins consisting in treating the skins with a mineral tanning solution mixed with a fermented solution of wheat flour, yeast, alcohol and water, substantially as herein described.

4. The process of tanning fur skins with 100 a mineral tanning solution mixed with a fermented organic solution of the ingredients and in about the proportions herein specified.

ROBERT NASSE.

Witnesses:

H. L. FISCHER,  
A. L. KRENICK.